

1

3,249,222

## METHOD OF SORTING OUT DEFECTIVE METALLIC RESISTORS BY SENSING THE CURRENT NOISE INDEX THEREOF

John G. Curtis, Bradford, Pa., assignor to Corning Glass Works, Corning, N.Y., a corporation of New York  
No Drawing. Filed Sept. 13, 1962, Ser. No. 223,520  
1 Claim. (Cl. 209—81)

This invention relates to a non-destructive method for sorting defective resistors from a quantity of resistors and more particularly to a method of determining defective resistors by measuring resistor current noise index.

The method of this invention is particularly suitable for sorting out defective metallic oxide film resistors. Such resistors are formed by applying a patterned metallic oxide film on a non-conductive substrate or a solid film which is thereafter patterned by spiralling or the like. For one example of a suitable film, its characteristics and method of application, reference is made to U.S. Patent No. 2,564,706 issued to John M. Mochel.

The quality of metallic oxide film or the like resistors is determined not only by the absolute resistance of the resistor and its closeness to the indicated nominal value thereof, but also by its temperature coefficient of resistance; load life test resistance drifts, that is the variation of resistance with time and load; power overload capability, and the like. Depending on the ultimate use of the resistors, various desired limits of acceptability are placed on the above-noted parameters. In the art, resistors which fall within the desired limits are termed acceptable or normal and those that fall outside of or exceed said limits are termed unacceptable, abnormal, or defective. In practice, determination of the temperature coefficient of resistance as well as the load life test resistance drift of a resistor is a tedious, time-consuming and costly procedure. In the case of the load life test it is also destructive. It, therefore, becomes impractical to measure these parameters on a 100 percent basis, and in the art they are in fact measured only on a sample basis which usually represents a small percentage of the total lot.

It has been found that metallic oxide film resistors fall outside acceptable limits of temperature coefficient of resistance and load life test resistance drift when they have certain structural and fabrication defects. Some of these defects are: film scratches, film porosity, checks or cracks in the non-conductive substrate, chips of the substrate, excessive end cap-to-film contact resistance, bridges of undisturbed film as well as bridges of foreign material across the cut path or in the current path of a spiralled resistor, and the like. It has been discovered that these structural and fabricating defects cause the resistor current noise index to rise substantially proportionately to the extent of said defects, that is, the greater number of said defects found on the resistor, as well as when such defects are more serious, the resistor current noise index is higher.

As used herein, resistor current noise is defined as unwanted or undesired resistance fluctuations between the resistor terminals while a constant flow of current is passed through the conductive portion of said resistor within a frequency band, the index of which is a function of the value of the intensity of the disturbance expressed in decibels by the relationship,

$$\text{noise index} = 20 \log \frac{uv}{V}$$

where  $uv$  is the noise voltage and  $V$  is the applied voltage.

2

It is an object of this invention to provide a non-destructive method of sorting out defective resistors rapidly and reliably.

It is another object of this invention to provide a method for rapidly sorting out resistors having an excessive temperature coefficient of resistance on a 100 percent basis.

It is still another object of this invention to provide a method for rapidly sorting out resistors having excessive load life resistance variations on a 100 percent basis.

Additional objects, features, and advantages of the present invention will become apparent, to those skilled in the art, from the following detailed description, where, by way of example, only the preferred embodiments of this invention are described.

According to the invention, resistors which are defective or unacceptable due to an excessive temperature coefficient of resistance or to excessive load life test resistance variations or drifts can be sorted out from a production run of resistors by determining the current noise index of such resistors which substantially corresponds to an acceptable limit of temperature coefficient of resistance and an acceptable limit of load life test resistance variation of such a type of resistor and thereafter rejecting all resistors of the same type having a current noise index higher than the determined value of noise index.

A typical example of carrying out the present invention is illustrated by the following description. A 100 piece sample lot of individually identified metallic oxide, spiral cut, film resistors, having a rating of  $\frac{1}{2}$  watt and 150K ohms, said film being of the type described in the heretofore noted Mochel patent, were selected for determining the current noise index limits. The normal performance of this type of resistor was predetermined to be as follows: A temperature coefficient of resistance of 150 parts per million per degree centigrade; a 1000 hour load life test resistance variation or drift ranging from approximately +0.2 to +0.6 percent.

The current noise index of each of the resistors in the sample lot was measured. Then the resistances of each of said resistors were measured at +25° C., -15° C., -55° C., +65° C., and +150° C. and the temperature coefficients were calculated as related to +25° C.

The current noise index was measured again. Thereafter, a 1000 hour cycled load life test was conducted and the resistance of each of said resistors was measured. It was found that all resistors having temperature coefficients greater than 150 parts per million per degree centigrade and resistance drifts greater than +0.2 to +0.6 percent had a current noise index exceeding -21.3 decibels.

A production run check of the same type of resistors, rejecting all resistors having a noise index higher than -21.3 decibels, would result in substantially rejecting all resistors having a temperature coefficient greater than 150 parts per million per degree centigrade and a load life test resistance drift greater than +0.2 to 0.6 percent.

It is readily seen that different types of resistors having different ratings and the like will cause the current noise index limit to vary accordingly, therefore, a noise index limit must be determined for each type of resistor. Furthermore, the current noise index limit will of course vary with the desired limits of temperature coefficients of resistance and load life test resistance drifts which are considered acceptable and normal. This will of course vary with the type and quality of resistor being produced.

Although the present invention has been described with respect to specific details of certain embodiments thereof, it is not intended that such details be limitations upon

the scope of the invention except insofar as set forth in the following claims.

What is claimed is:

A method of sorting metallic oxide film resistors exceeding acceptable values of temperature coefficient of resistance and load life test resistance drift comprising the steps of

providing a supply of resistors,

selecting maximum acceptable values of temperature coefficient of resistance and resistance drift of said resistors,

selecting a sample lot from said supply of resistors, applying electrical energy to said sample lot of re-

sistors while quantitatively sensing the current noise index thereof, quantitatively sensing in any order the resistance and temperature of said sample lot of resistors to obtain the load life test resistance drift, and the temperature coefficient of resistance thereof,

selecting a maximum acceptable value of current noise index which is equivalent to said maximum acceptable values of temperature coefficient of resistance and resistance drift,

applying electrical energy to the remaining resistors of said supply of resistors while sensing the current noise index thereof, and

rejecting those resistors having a current noise index exceeding said acceptable value of current noise index.

References Cited by the Examiner

UNITED STATES PATENTS

1,931,054 10/1933 Butterfield 324—62

WALTER L. CARLSON, *Primary Examiner*.

CLAUDE A. S. HAMRICK, EDWARD E. KUBASIEWICZ, *Assistant Examiners*.